

United States Patent [191]  
Stack

[11] 3,884,736  
[45] May 20, 1975

[54] **DOUBLE-BASE PROPELLANT  
CONTAINING AN AROMATIC HYDROXY  
COMPOUND**

[75] Inventor: Joseph S. Stack, Riverdale, N.J.

[73] Assignee: The United States of America as  
represented by the Secretary of the  
Army, Washington, D.C.

[22] Filed: Apr. 6, 1967

[21] Appl. No.: 630,490

[52] U.S. Cl. .... 149/100; 149/19.8; 149/38;  
149/42; 149/44; 149/76; 149/92; 149/98

[51] Int. Cl. .... C06b 5/00

[58] Field of Search .... 149/94, 95, 96, 98, 19,  
149/38, 100, 42, 44, 18, 19, 20, 19.8, 76, 92

[56] **References Cited**  
**UNITED STATES PATENTS**

|           |         |                 |       |          |
|-----------|---------|-----------------|-------|----------|
| 3,002,830 | 10/1961 | Barr            | ..... | 149/19   |
| 3,132,976 | 5/1964  | Klager et al.   | ..... | 149/19   |
| 3,141,294 | 7/1964  | Lawrence et al. | ..... | 149/19   |
| 3,215,573 | 11/1965 | Winkler         | ..... | 149/19 X |
| 3,245,849 | 4/1966  | Klager et al.   | ..... | 149/19   |
| 3,260,631 | 7/1966  | Witz et al.     | ..... | 149/19   |
| 3,296,043 | 1/1967  | Fluke et al.    | ..... | 149/19   |

*Primary Examiner—Stephen J. Lechert, Jr.  
Attorney, Agent, or Firm—Nathan Edelberg; Robert P.  
Gibson; A. Victor Erkkilla*

**EXEMPLARY CLAIM**

1. In a double base plastisol type propellant containing nitrocellulose and liquid nitrate esters in combination with between 0.5 and 2.0 percent by weight of either 2,4-tolylene diisocyanate or hexamethylene diisocyanate based on the weight of said propellant, the improvement consisting in the incorporation of between 0.5 and 2.0 percent by weight of an aromatic hydroxy compound based on the weight of said diisocyanate, thereby rendering said propellant homogeneous and void-free, said aromatic hydroxy compound selected from the group consisting of  
1,3-dihydroxy benzene,  
1,2-dihydroxy benzene,  
1-methyl-3,5-dihydroxy benzene,  
1,4-dihydroxy benzene,  
1,2,3-trihydroxy benzene,  
1,3,5-trihydroxy benzene,  
1,3-dihydroxy-2-nitro-benzene,  
1-hydroxy-3-aceto-benzene,  
1,3-dihydroxy-2-methyl benzene,  
1-methanol-2-hydroxy benzene, and  
1,3-dihydroxy-2,4-nitroso-benzene.

**16 Claims, 2 Drawing Figures**

PATENTED MAY 20 1975

3,884,736



FIG. 1  
(PRIOR ART)

FIG. 2



INVENTOR  
JOSEPH S STACK

# 1

## DOUBLE-BASE PROPELLANT CONTAINING AN AROMATIC HYDROXY COMPOUND

This invention relates to a porous free diisocyanate treated nitrocellulose based plastisol propellant.

In the past, one of the major disadvantages of conventional composite nitrocellulose based plastisol type propellants was the inability to be procured in a variety of formulations. It was found that such systems, which had favorable mechanical properties over a wide range of temperature extremes, could only be formulated over a narrow range of ratios with respect to their ingredients. As a result, the variety of formulations which could be prepared of a system containing a specific ingredient such as a high energy casting solvent was very much limited.

When the above systems were crosslinked with diisocyanate containing materials, the operating range over which the propellant exhibited favorable mechanical properties was expanded considerably. It was apparent that the diisocyanate treatment created a versatility of formulations for the composite nitrocellulose based plastisol systems which heretofore could not be achieved with conventional systems which were untreated.

As a further extension of the above, it was found that diisocyanate containing compounds were quite useful in the improvement of the physical properties of the nitrocellulose based plastisol propellants. It is thought that this is due to the reactivity of the diisocyanate containing material with such propellant ingredients as nitrocellulose, amines, and the hydroxy containing compounds. As a result of this action, the physical properties of the propellant such as elongation and tensile strength are improved to a degree beyond that of the base propellant. This is quite useful because, as an example, castable case-bondable nitrocellulose based plastisol propellants are desired which possess adequate elongation at low temperatures in order to withstand the thermal stresses created between the propellant and the rocket motor case. Further, propellants with sufficient rigidity and strength at high temperatures, such as the above diisocyanate treated propellant, are necessary to prevent damaging deformation of the propellant during storage and firing.

However, even though the treatment of nitrocellulose based plastisol propellants with diisocyanate containing materials is accompanied by improvement in physical properties, there is one serious problem. The diisocyanate containing materials in use today are highly reactive with water. They react with even trace amounts of moisture present in the composite double-base propellant to produce carbon dioxide which, in turn, leads to the formation of a porous system during subsequent processing and curing of the propellant. Thus, a propellant is produced which possesses a multitude of void-like pores. As a practical matter, it has thus been found difficult to duplicate or control the burning characteristics of a porous diisocyanate treated nitrocellulose based plastisol propellant. As a result, this adversely affects the reliability of the ballistics

characteristics of the propellant. However, it has been found that, in some cases, void free and homogeneous propellants might be prepared by employing meticulous drying and handling of ingredients and tedious procedures to avoid the presence of water in the system. As is apparent, such techniques are highly dangerous. Thus, in view of the above, the propellant formulator is confronted with a difficult problem when processing such propellants by standard processing techniques.

10 This invention provides the needs of the art, as heretofore set forth, by a simple technique which allows the production of void-free diisocyanate treated nitrocellulose based plastisol, with their attendant advantages, by existing facilities and operating procedures.

15 An object of this invention is to provide a homogeneous, porous free, diisocyanate treated nitrocellulose based plastisol propellant.

Another object is to provide the propellant described by existing facilities and operating procedures.

20 Other objects and many of the attendant advantages of this invention will be readily appreciated as the same become better understood by reference to the following detailed description when considered in connection with the accompanying pictorial showing wherein:

25 FIG. 1 is a pictorial view of a conventional diisocyanate treated nitrocellulose based plastisol propellant.

FIG. 2 is a pictorial view of the formulation of FIG. 1 which has been modified in accordance with this invention.

30 It has now been discovered that if a slight amount of an aromatic hydroxy containing compounds such as 1,3-dihydroxy benzene, otherwise known as resorcinol, is added to the propellant during processing, a homogeneous porous free diisocyanate treated nitrocellulose based plastisol propellant may be produced utilizing conventional facilities and operating procedures. The grain structure of such a propellant is illustrated in the photograph of FIG. 2. However, in contrast, as shown in the photograph of FIG. 1, the grain structure of the conventional diisocyanate treated nitrocellulose based plastisol propellant produced by the same procedures is non-homogeneous and has a multitude of void-like spaces throughout its mass. This is clearly an achievement in view of the fact that conventional procedures are utilized throughout the treatment of the propellant with both the diisocyanate containing material and the aromatic hydroxy compound.

35 The aromatic hydroxy compounds which may be utilized in this invention to give results comparable to 1,3-dihydroxy benzene include: 1,2-dihydroxy benzene; 1-methyl - 3,5-dihydroxy benzene; 1,4-dihydroxy benzene; 1,2,3-trihydroxy benzene; 1,3,5-trihydroxy benzene; 1,3-dihydroxy - 2 - nitro-benzene; 1-hydroxy - 3-aceto-benzene; 1,3-dihydroxy - 2-methyl benzene; 1-methanol - 2-hydroxy benzene, and 1,3-dihydroxy - 2,4-nitroso-benzene. All of the above aromatic hydroxy compounds give similar results when utilized to modify the diisocyanate treated nitrocellulose based plastisol propellant.

40 45 50 55 60 65 Typical nitrocellulose based plastisol propellant formulations embodying the concept of this invention include the following set forth in Table 1 below.

TABLE 1

| INGREDIENTS                 | 1    | 2    | 3    | 4    | 5    | 6    |
|-----------------------------|------|------|------|------|------|------|
| Fluid Ball Powder, 2159 (1) | 15.5 | 18.5 | 20.5 | 22.5 | 27.5 | 31.5 |
| Fluid Ball Powder, 2014 (2) | 1.0  | 1.0  | 1.0  | 1.0  | 1.0  | 1.0  |
| Aluminum, Reynolds 6073     | 1.00 | 1.00 | 1.00 | 1.00 | 1.00 | 1.00 |

TABLE I - Continued

| INGREDIENTS                      | 1                 | 2        | 3    | 4     | 5    | 6    |
|----------------------------------|-------------------|----------|------|-------|------|------|
| Ammonium Perchlorate, 5074       | 21.0              | 21.0     | 21.0 | 21.0  | 21.0 | 21.0 |
| Resorcinol, added                | 2.0               | 2.0      | 2.0  | 2.0   | 2.0  | 2.0  |
| 2,4-tolylene diisocyanate, added | 1.24              | 1.47     | 1.62 | 1.77  | 2.15 | 2.38 |
| Casting Solvent "X" (3)          | 49.5              | 46.5     | 44.5 | 42.5  | 37.5 | 33.5 |
| Powder/Solvent Ratio             | 0.33              | 0.42     | 0.49 | 0.556 | 0.77 | 0.99 |
| NOTE:                            | Percent by Weight |          |      |       |      |      |
| Compositions of Ball Powder      | 2159 (1)          | 2014 (2) |      |       |      |      |
| (a) Nitrocellulose, 12.6% N.     | 90.0              | 74.0     |      |       |      |      |
| (b) Nitroglycerin                | 8.0               | 24.0     |      |       |      |      |
| (c) 2-nitrodiphenylamine         | 2.0               | 2.0      |      |       |      |      |
| Casting Solvent X (3)            | Percent by weight |          |      |       |      |      |
| (a) Triethylene glycol dinitrate | 65%               |          |      |       |      |      |
| Butane Triol Trinitrate          | 34%               |          |      |       |      |      |
| 2-nitrodiphenylamine             | 1%                |          |      |       |      |      |

The formulations set forth above all exhibit the improvement of mechanical properties heretofore described in connection with the crosslinking of the base propellant with a diisocyanate containing material. In addition, the final cast of the composites set forth in Table I all resemble the pictorial view set forth in FIG. 2 in that they are homogeneous and void free. All of the above formulations were processed in accordance with the procedure set forth in Example 1 below:

#### EXAMPLE I

The fluid ball powder and resorcinol is added to the casting solvent dehydrated to a moisture content of approximately 0.1 percent and is left at about  $70^{\circ}\pm 5^{\circ}\text{F}$  for about 18 hours. At the end of this period, the aluminum and ammonium perchlorate ingredients are added to the resulting solution accompanied by agitation. To the above, the diisocyanate containing material is added and the mass is mixed for about 1 hour under a vacuum of 4 to 10 mm of mercury. The mass is mixed until a viscosity of 30,000 to 40,000 centipoise is reached at which time the mass is cast into the desired molds and cured at  $60^{\circ}\text{C}$  for 3 days.

Although there are many diisocyanate containing materials which may be utilized to modify the nitrocellulose based plastisol propellant, the most common are 2,4-tolylene diisocyanate and hexamethylene diisocyanate. In general, the amount of diisocyanate containing material utilized in the treatment of the described composite propellant may vary from 0.5 to 5.0 percent by weight based on the weight of the propellant. Generally, the amount of diisocyanate containing materials utilized in the system varies with the amount of nitrocellulose in the propellant. The most effective concentration of diisocyanate containing material has been found to be between 0.5 and 3.0 percent. In the latter range, the modified or cross-linked nitrocellulose based plastisol propellant exhibits exceptional improvement in mechanical properties consistent with the desired degree of homogeneity. At concentrations of less than 0.5 percent, there is only marginal improvement in the mechanical properties when contrasted to the uncross-linked propellant composite. At concentrations of over 3.0 percent, the propellant tends to exhibit brittleness as a result of the high degree of crosslinking of the propellant. In addition, the propellant may have a non-homogeneous appearance. As noted, the crosslinking agent varies with the amount of nitrocellulose in the propellant. In the composites set forth in Table I, the ball powder contains between 74 and 90 percent by

weight of nitrocellulose based on the overall weight of the ball powder.

Also, in general, the amount of aromatic hydroxy compound employed in a diisocyanate treated nitrocellulose based plastisol propellant varies with the amount of diisocyanate utilized in the system. In accordance with this concept, the following table is submitted.

TABLE II\*

|    | Diisocyanate | Aromatic Hydroxy Compound |
|----|--------------|---------------------------|
| 30 | 0.5 - 0.75   | 0.5                       |
|    | 0.76 - 1.5   | 1.0 - 1.5                 |
|    | 1.5 - 2.0    | 2.0                       |
|    | > 2.0        | 2.0                       |

\*All figures represent per cent by weight.

The above table sets forth the amount of aromatic hydroxy compound utilized in a propellant system based on the amount of diisocyanate containing material utilized to crosslink the propellant composite. If an amount of hydroxy compound below 0.5 percent is utilized, the propellant will exhibit a low degree of elongation and high degree of tensile strength. However, the overall system will be void free but thermal stability will be borderline. At hydroxy compound concentrations of 1.0 to 1.5 percent, the propellant systems are void free accompanied by reasonably good mechanical properties and good thermal stability. At the 2.0 percent concentration of the hydroxy compound, the optimum in mechanical properties and thermal stability is obtained with the treated propellant system. If amount above 2 percent is utilized, the propellant exhibits a low degree of tensile strength and a high degree of elongation. It has been found that within the range indicated, the overall stability of the propellant is excellent and the treated propellant is homogeneous and void free.

As is evident from the above, aromatic hydroxy compounds, when employed in small concentrations in the described plastisol type propellants, control the gassing of carbon dioxide which is normally associated with systems cross-linked with 2,4-tolylene and hexamethylene diisocyanate. As a result, it is now possible to process homogeneous and void free composite nitrocellulose based plastisol propellant under non-rigidly controlled environments and without meticulous drying of special ingredient in the composite.

Obviously, there are many modifications and variations of the present invention which are possible in light of the above teachings. It is therefore to be understood that within the scope of the appended claims, the in-

vention may be practiced otherwise than as specifically described.

I claim:

1. In a double base plastisol type propellant containing nitrocellulose and liquid nitrate esters in combination with between 0.5 and 2.0 percent by weight of either 2,4-tolylene diisocyanate or hexamethylene diisocyanate based on the weight of said propellant, the improvement consisting in the incorporation of between 0.5 and 2.0 percent by weight of an aromatic hydroxy compound based on the weight of said diisocyanate, thereby rendering said propellant homogeneous and void-free, said aromatic hydroxy compound selected from the group consisting of

1,3-dihydroxy benzene,  
1,2-dihydroxy benzene,  
1-methyl-3,5-dihydroxy benzene,  
1,4-dihydroxy benzene,  
1,2,3-trihydroxy benzene,  
1,3,5-trihydroxy benzene,  
1,3-dihydroxy-2-nitro-benzene,  
1-hydroxy-3-aceto-benzene,  
1,3-dihydroxy-2-methyl benzene,  
1-methanol-2-hydroxy benzene, and  
1,3-dihydroxy-2,4-nitroso-benzene.

2. In the propellant of claim 1 wherein said diisocyanate is present in an amount between 0.5 and 0.75 percent by weight, the improvement wherein said propellant is modified with 0.5 percent by weight of said aromatic hydroxy compound.

3. In the propellant of claim 1 wherein said diisocyanate is present in an amount between 0.76 and 1.5 percent by weight, the improvement wherein said propellant is modified with between 1.0 and 1.5 percent by weight of said aromatic hydroxy compound.

4. In the propellant of claim 1 wherein said diisocyanate is present in an amount between 1.5 and 2.0 percent by weight, the improvement wherein said propellant is modified with 2.0 percent by weight of said aromatic hydroxy compound.

40

5. In the propellant of claim 1 wherein said diisocyanate is present in an amount of 2.0 percent by weight, the improvement wherein said propellant is modified with 2.0 percent by weight of said aromatic hydroxy compound.

6. In the propellant of claim 1, the improvement wherein said propellant is modified with 1,3-dihydroxy benzene.

7. In the propellant of claim 1, the improvement wherein said propellant is modified with 1,2-dihydroxy benzene.

8. In the propellant of claim 1, the improvement wherein said propellant is modified with 1-methyl-3,5-dihydroxy benzene.

9. In the propellant of claim 1, the improvement wherein said propellant is modified with 1,4-dihydroxy benzene.

10. In the propellant of claim 1, the improvement wherein said propellant is modified with 1,2,3-trihydroxy benzene.

11. In the propellant of claim 1, the improvement wherein said propellant is modified with 1,3,5-trihydroxy benzene.

12. In the propellant of claim 1, the improvement wherein said propellant is modified with 1,3-dihydroxy-2-nitro-benzene.

13. In the propellant of claim 1, the improvement wherein said propellant is modified with 1-hydroxy-3-aceto-benzene.

14. In the propellant of claim 1, the improvement wherein said propellant is modified with 1,3-dihydroxy-2-methyl benzene.

15. In the propellant of claim 1, the improvement wherein said propellant is modified with 1-methanol-2-hydroxy benzene.

16. In the propellant of claim 1, the improvement wherein said propellant is modified with 1,3-dihydroxy-2,4-nitroso-benzene.

\* \* \* \* \*

45

50

55

60

65